

April 12, 1938.

J. O. BETTERTON ET AL.

2,113,643

## PROCESS FOR TREATING METALS

Filed May 27, 1935



INVENTORS  
*Jesse O. Betterton*  
BY *Albert J. Phillips*  
*James K. Kent*  
ATTORNEY

## UNITED STATES PATENT OFFICE

2,113,643

## PROCESS FOR TREATING METALS

Jesse O. Betterton and Albert J. Phillips, Metuchen, N. J., assignors to American Smelting and Refining Company, New York, N. Y., a corporation of New Jersey

Application May 27, 1935, Serial No. 23,577

12 Claims. (Cl. 75—63)

In accordance with the present invention, there is provided an improved process for separating tin from tin containing alloys, especially tin-lead alloys and lead alloys containing tin.

5 In salvaging scrap lead and drosses arising from various alloying procedures, lead and lead alloys containing substantial amounts of tin are produced. While it is usually a fairly simple matter to remove tin from these alloys by oxidation, such procedure is open to the objection that there is not obtained a clean-cut separation of tin from the lead. Usually a rather large amount of lead is taken off with the oxidized dross, and the material produced from this dross 10 is often so rich in lead as to necessitate re-concentration in order to produce a readily salable lead-tin alloy. In addition, certain tin containing alloys of lead such as lead-antimony alloys, for example, are not susceptible to the oxidation procedure for removing their tin content without involving a considerable and undesirable loss of antimony from the lead, and at the same time producing a tin concentrate relatively rich in antimony, which involves elaborate reprocessing operations in order to make satisfactory 15 separations.

20 One of the objects of the present invention is to provide a process for separating the tin from alloys such as those above mentioned in which the tin is substantially completely removed from the alloy in a simple and direct operation.

25 A still further object of the invention is to provide a process for removing tin from lead-tin alloys, and tin-containing alloys of lead wherein there is produced a tin compound substantially free from other base metals from which a tin of very high purity may be produced.

30 A still further object of the invention is to provide a process of the above indicated character in which there are avoided any substantial losses of lead or of any of the usual metals alloyed with lead.

35 Other objects of the invention will appear hereinafter, the novel features and combinations of steps of the new process being set forth in the appended claims.

40 The present invention depends upon the facts, first, that tin in the presence of lead chloride acts as a reducer for the latter to form stannous chloride in accordance with the reaction



45 and, second, that the resulting stannous chloride is converted into stannic chloride by chlorine gas:



The stannic chloride, being volatile at the temperatures employed, passes out from the system.

The first of these reactions is a simple equilibrium, as indicated above, and the equilibrium point favors a predominance of lead over tin, since the heat of formation of lead chloride is somewhat higher than that of stannous chloride. Therefore, when it is attempted to carry out the above reaction, only a small amount of tin will react with lead chloride to form stannous chloride; if, however, the tin in the form of chloride be continuously removed from the reaction system, as takes place upon its conversion into stannic chloride, the reduction of the lead 15 chloride will proceed to completion. As the stannic chloride volatilizes from the reaction system, additional tin is removed by reaction with the lead chloride, and there is obtained, in effect, the selective chloridization of the tin from the lead.

In carrying out the above indicated reaction, the lead alloy containing tin is melted, and the resulting molten bath is skimmed free from oxide products. Lead chloride is charged onto the surface of the bath, the lead chloride being preferably mixed with suitable salts which will lower the melting point of the lead chloride without entering the reaction. Alkali and alkaline earth chlorides, such as sodium chloride, potassium chloride, and calcium chloride have been employed, and many others may be used likewise. The result is that upon the molten alloy bath there is floating a layer of molten slag, comprising, principally, lead chloride. A layer of such slag of considerable depth is allowed to form there being a partial interaction of the tin in the alloy bath with the lead chloride of the slag in accordance with the first equation above. In order to remove the resulting stannous chloride, thereby enabling the reaction to run to completion, chlorine gas is passed through the molten slag layer, care being taken to avoid contact between the chlorine and the alloy bath, the latter being stirred vigorously, however, to promote contact between the metal bath and the molten salt slag. During this operation, stannic chloride is evolved freely from the slag, and may be condensed and recovered. By maintaining the chlorine out of contact with the molten metal bath, formation of lead chloride from the lead is avoided, the lead chloride in the slag being reduced to metallic lead by interfacial reaction with tin in the metal bath, so that in continued commercial operations it is necessary to occasion- 55

ally introduce chlorine into the lead bath in order to regenerate the lead chloride of the slag layer for replacing that which has been removed by the aforesaid reduction. The chlorination of the slag may be carried out either continuously or intermittently, one of the principal features to be observed being to maintain the chlorine gas out of contact with the alloy bath except as is necessary to replenish the chloride content of the slag as explained above and to control admission of chlorine at such rate as will enable the chlorine to combine substantially completely with the stannous chloride in the slag except during the intervals of intermittent introduction into the bath.

The accompanying drawing illustrates forms of apparatus which may be employed in carrying out the process of the present invention. In the drawing—

20 Fig. 1 is a diagrammatic sectional elevation illustrating one form of apparatus which may be employed for the purpose;

25 Fig. 2 is a similar view showing a somewhat different form of apparatus.

30 Referring more particularly to the drawing, and to Fig. 1, it will be seen that the materials are received in a receptacle 1, which may be of any suitable material such as cast iron, and which may be provided with a flange 2 for supporting the receptacle 1 in a suitable furnace 3, provided with one or more burners 4 for melting the charge in the receptacle 1. The receptacle 1 is provided with a tightly fitting cover 5 suitably apertured to receive a stirring device 6, a condenser 7, which 35 is water cooled, and a tube or pipe 8 for the admission of chlorine gas. The stirrer 6 has a stem 9, which is mounted in a bearing 10 in the cover 5, and also in a bearing 11 supported on the cover 5 by brackets 12 and 13. The stem 9 terminates in a pulley 13a, around which is passed a driving belt 14 which is driven from a suitable motor, not shown.

40 The charge of metal or alloy from which the tin is to be separated is placed in the receptacle 1, as indicated at 15, and this charge is melted. The salts to form the slag layer are distributed over the metal to form a layer 16 of substantial depth, and because of its lower specific gravity, this layer will float upon the charge of metal. Where the metal charge 15 is a lead-tin alloy, or a lead alloy containing tin, the layer 16 is principally lead chloride, although there may be mixed therewith suitable fluxing materials, chemically inert under the conditions of operations, which will lower the melting point of the salt slag and enable the operations to be carried out at lower temperatures than would be feasible were these fluxes omitted. As indicated above, alkali or alkaline earth chlorides are suitable 45 fluxing materials.

50 When the entire charge in the receptacle 1 has been melted, the cover 5 is placed in position, and the chlorine inlet 8 and condenser 7 positioned and connected to the cover 5, it being understood that all connections are gas-tight to avoid leakage. The chlorine inlet 8 dips beneath the salt slag layer 16, but terminates above the metal layer 15, so as to prevent contact between the chlorine entering the charge through the inlet 8 and the 55 metallic layer 15. Chlorine is gently bubbled through the salt slag layer, the entire charge being maintained molten, and the layer 15 is agitated by stirring with the stirrer 6 so as to bring the metals of the layer 15 into contact with the 60 fused salt layer 16. The tin in the metallic layer

15 reacts with the lead chloride in the layer 16 to form stannous chloride which remains in the salt slag layer 16, but which is quickly converted into stannic chloride by action of the chlorine bubbling through the salt slag layer 16. The stannic chloride thus produced is volatile at the temperatures of operation, and passes into the condenser 7 where the vapors are condensed, and the resulting liquid stannic chloride recovered. The chlorine may be introduced continuously or intermittently, as desired, in view of the particular operating conditions present.

10 As a specific illustration of the operation of the present process, it may be mentioned that 500 gms. of lead alloy containing 5% tin were melted in the receptacle 1, and the small amount of oxide dross arising from the melting operation was carefully removed. To the molten alloy charge were added 448 gms. of lead chloride containing 39 gms. of sodium chloride to suitably lower the 15 melting point of the salt slag. The salt mixture was charged on top of the metallic charge and heated until the entire charge was fully molten. Chlorine was then gently bubbled through pipe 20 8, care being taken that chlorine did not enter the metallic layer 15 and to control the bubbling so that the rate of bubbling was such that the chlorine combined substantially entirely with the stannous chloride. This metallic layer 15 was 25 suitably agitated, and the fume evolved during the reaction was condensed in the condenser 7, and collected in a suitable receptacle not shown. Practically pure stannic chloride was collected during a period of about one-half hour, which 30 stannic chloride showed by chemical analysis, a 35 tin content of 21.22 gms. of tin. At the end of one-half hour, the rate of evolution of stannic chloride was so small that the chlorination was discontinued. There were recovered 502 gms. of metal from the charge, the excess weight representing lead entering the charge from the reduction of the lead chloride in the slag during the process. The metal contained only 0.18% of tin. The slag contained 0.55% tin and weighed approximately 450 gms.

40 In another run, 78 1/4 pounds of lead alloy containing 3% of tin were melted in the kettle or receptacle 1. To the molten charge was added a salt slag containing 40 pounds of lead chloride, 3.2 pounds of sodium chloride, and 2 pounds of 45 potassium chloride, the temperature being increased until the entire charge was liquid. The stirrer 6 was introduced into the molten metal, and the cover 2 placed in position on the receptacle 1, together with the condenser 7 and chlorine pipe or tube 8, the latter being inserted so 50 that the chlorine entered the slag about one inch above the metal line. During a period of three hours, 2.7 pounds of chlorine were introduced into the molten slag, producing approximately 500 c. c. 55 of stannic chloride. At the end of the run, the metal in the bath weighed slightly more than 76 pounds and contained 0.52% of tin. The slag weighed 43 pounds, and contained 1.5% of tin.

60 It will be understood, of course, that the tin content of the recovered stannic chloride may be recovered by any of the well-known operations, or the stannic chloride may be marketed as such, if so desired.

65 The apparatus shown in Fig. 2 operates similarly to that shown in Fig. 1. The receptacle 1, Fig. 2, may be a cast iron kettle, provided with a flange 2 for supporting the kettle 1 in the furnace 3, as described in connection with Fig. 1. One or more burners 4 may be employed to heat 70

the furnace 3. The metal charge 15 is placed in the receptacle 1 and melted, and a cylinder 17 is vertically lowered into the receptacle. The lower end 18 of the cylinder is open, and is positioned beneath the surface of the metal charge, the upper end 19 of the cylinder being closed. The end 19 of the cylinder 17 is adapted to receive a nozzle 20 communicating with a chlorine line 21 coming from a suitable source of chlorine, not shown. The nozzle 20 is restricted at 21a to produce a vortex action. A pump 22 is adapted to pump the molten salt slag 16, as described above, up through pipe 23 and into the nozzle 20, where it is mixed with the incoming chlorine, and the stannous chloride in the slag is thereby converted into stannic chloride, which is then condensed in condenser 7, as above. The molten salt slag collects in a column 24 in the cylinder 17 until the weight of this column forces the salt slag out through the open end 18 and into the metal charge, the salt slag rising through the metal to the surface thereof, whence it is recirculated by the pump 22 as previously described. As the molten salt slag passes from the open end 18 of the cylinder 17 upwardly through the metal layer 15, the reduction of the lead chloride in the slag by the tin in layer 15 is initiated, the resulting stannous chloride being converted into volatile stannic chloride in the nozzle 20 and cylinder 17. The vortex action of the nozzle 20 materially facilitates the contact between the molten slag and the chlorine entering the nozzle 20 through the pipe 21 thus increasing the efficiency of the conversion of the stannous chloride into stannic chloride, and therefore increases the rate at which the tin is removed from the metal bath 15.

It will be noted that when alloys of lead are being treated for the removal of tin therefrom, it is preferred, of course, to use lead chloride as the active ingredient in the fused salt slag, since such avoids the possibility of introducing any metal other than lead into the metallic bath, it being remembered that as the tin is removed from the reaction system, the active chloride is reduced to metal, which enters the metallic bath. So far as concerns the operativeness of the process, however, other chlorides reducible by tin may be employed, such as, for example, chlorides of metals electronegative to tin.

Attention is called to the fact that the active ingredient in the slag is selected to be such as to be reacted upon by the metallic constituent in the bath which is to be removed from the bath, the resulting compound of that metallic constituent being removable readily from the reaction system so that the desired conversion and removal can proceed to completion, it being desired to embrace within the scope of this invention such modifications and changes as may be desirable or necessary to adapt it to varying conditions and uses.

What is claimed is:

1. The process of removing tin from a lead or alloys of lead containing tin which comprises forming a molten bath thereof, overlying the said bath with a layer of molten slag containing principally lead chloride, contacting the bath and slag until a reduction by the tin is initiated so that at least a small amount of stannous chloride is included in the slag, passing chlorine gas into the slag to convert the stannous chloride into stannic chloride intercirculating the slag and the metal bath while continuing to chloridize the slag to maintain reactive interfacial contact

between the slag and the bath for maintaining continuously a tin content in the slag, allowing the stannic chloride to volatilize from the slag, thereby substantially completely removing the tin from the bath, and regenerating the chloride content of the slag as it becomes depleted by periodically introducing chlorine into the metal bath.

2. The process of removing tin from lead or alloys of lead containing tin which comprises forming a molten bath thereof, overlying the said bath with a layer of molten slag containing principally lead chloride, circulating the slag through the metal to intimately contact the bath and the slag to effect an initiation of reduction of the lead chloride by the tin so that at least a small amount of stannous chloride is included in the slag, chlorinating the slag to convert the stannous chloride into stannic chloride by passing chlorine into the slag while avoiding substantial contact between the chlorine and the bath notwithstanding the circulation of the slag through the bath, allowing the stannic chloride to volatilize from the slag, thereby substantially completely removing the tin from the bath, intermittently passing chlorine into the said bath to regenerate the lead chloride content of the slag as it becomes depleted, and condensing and recovering the stannic chloride evolved from the slag.

3. The process of detinning tin-bearing lead and lead alloys which comprises melting the lead and lead alloys in a suitable receptacle under a layer of slag comprising at least relatively large proportions of lead chloride, inserting into the receptacle and through the slag a reaction vessel having an open end so that the said open end is below the metal level in the receptacle, continuously pumping slag from the slag layer into the reaction vessel while admitting chlorine thereto to intimately contact the slag and chlorine while effecting displacement of metal from the interior of the reaction vessel, causing the chlorine treated slag to pass from the receptacle through the open end thereof and thence upwardly through the metal layer and in contact therewith, for recirculation through the reaction vessel, and recovering the stannic chloride produced in the reaction vessel.

4. The process of making stannic chloride which comprises continuously circulating molten stannous chloride-bearing material through a reaction vessel in contact with a stream of chlorine continuously passing into the vessel, intermixing the said material and the chlorine by a vortex action, continuously withdrawing stannic chloride from the reaction vessel, continuously replenishing the stannous chloride content of the residual material and continuously recycling the material through the reaction vessel in contact with fresh quantities of chlorine.

5. The process of recovering tin from tin-containing metals such as tin-containing lead and tin-containing lead alloys which comprises melting the metal under a layer slag containing lead chloride under conditions effecting a partial replacement of the lead of the lead chloride with tin thereby forming stannous chloride in the slag, confining a portion of the slag in a reaction vessel and contacting the said confined slag portion with chlorine to effect a production of stannic chloride, allowing the stannic chloride to separate from the confined slag portion, passing the said slag portion remaining after the chlorine treatment from the reaction vessel

through the metal to replenish the tin content of the slag, and recirculating the replenished slag through the reaction vessel in contact with fresh quantities of chlorine.

5 6. A process of detinning tin-containing metals which comprises chlorinating a molten stannous chloride-lead chloride-containing slag to continuously evolve stannic chloride therefrom while intercirculating the slag with a bath of tin-  
10 containing metal to maintain a tin content in the slag, and replenishing the lead chloride content of the slag from the bath as it becomes depleted, thereby maintaining the ability of the slag to pick up tin from the bath while avoiding  
15 formation of excessive amounts of lead chloride in the slag.

7. A process of detinning lead-tin alloys which comprises forming a molten bath thereof under a slag containing lead tin chlorides, reactively  
20 contacting the slag and bath to cause the slag to pick up tin from the bath while chloridizing the slag to evolve stannic chloride therefrom as the tin enters the slag, and periodically renewing the lead content of the slag as it becomes  
25 depleted thereby maintaining the reactivity of the slag with respect to the bath while avoiding building up excessive amounts of lead chloride therein.

8. A process of detinning lead-tin alloys which  
30 comprises forming a molten bath thereof under a slag containing lead and tin chlorides, continuously reactively contacting the slag and bath to cause the slag to pick up tin from the bath while continuously chloridizing the slag only to  
35 evolve stannic chloride therefrom as the tin enters the slag, and occasionally chloridizing the bath to renew the lead chloride content of the slag as it becomes depleted thereby maintaining the reactivity of the slag with respect to the  
40 bath while avoiding building up excessive amounts of lead chloride therein with consequent depletion of the lead in the bath.

9. A process for removing tin from lead-tin alloys which comprises forming a molten bath  
45 of the alloys, providing a molten slag cover for the bath comprising essentially lead chloride, intercirculating the slag and metal bath to effect a partial conversion of the lead chloride into stannous chloride by reaction at the liquid  
50 interface of the slag and metal between lead chloride of the slag and tin in the metal bath, and removing the tin from the slag as stannic chloride by passing controlled amounts of chlorine into the slag only at such a rate that the

chlorine combines substantially entirely with the stannous chloride in the slag.

10. A process for removing tin from alloys of tin and lead which comprises fusing the alloys to form a molten bath thereof, extracting tin therefrom in a fused chloride slag having a high content of lead chloride, removing the tin from the slag by passing controlled amounts of chlorine into the slag only at such rate that the chlorine combines substantially entirely with the stannous chloride in the slag, and replenishing the tin content of the slag from the tin in the bath being detinned by intercirculating the slag and metal to effect a reaction between lead chloride and tin at the interface between the slag and metal bath while continuing to pass the said controlled amounts of chlorine into the slag.

11. A process for removing tin from alloys of tin and lead which comprises forming a molten bath of the alloys, extracting tin therefrom in a fused chloride slag having a high content of lead chloride, removing the tin from the slag by passing controlled amounts of chlorine into the slag only at such rate that the chlorine combines substantially entirely with the stannous chloride in the slag, and replenishing the tin content of the slag from the tin in the bath being detinned by intercirculating the slag and metal to effect a reaction between lead chloride and tin at the interface between the slag and metal bath.

12. A process for removing tin from lead-tin alloys which comprises forming a molten bath of the alloys, providing for the bath a molten slag layer comprising essentially lead chloride on the metal bath, reactively contacting the slag and metal bath to effect a partial conversion of the lead chloride into stannous chloride by causing displacement of the lead from the lead chloride by tin in the bath, removing the tin from the slag as stannic chloride by passing controlled amounts of chlorine into the slag only at such rate that the chlorine combines substantially entirely with the stannous chloride in the slag, intercirculating the metal bath and slag to replenish the tin content of the slag as the tin is evolved therefrom by effecting interaction between lead chloride and tin at the interfacial surfaces between the bath and slag while continuing to pass the said controlled amounts of chlorine into the slag, and intermittently passing chlorine into the metal bath beneath the slag to regenerate the lead chloride content of the slag.

JESSE O. BETTERTON.

ALBERT J. PHILLIPS.

55